

BEST AVAILABLE COPY

UNITED STATES PATENT OFFICE.

HARRY W. BROADY, OF BAYSIDE, NEW YORK, ASSIGNOR TO THE LUNDIN COMPANY, INC., OF LONG ISLAND CITY, NEW YORK, A CORPORATION OF NEW YORK.

PROCESS AND PRODUCT OF TREATING WOOD.

1,203,577.

Specification of Letters Patent. Patented Nov. 7, 1916.

No Drawing.

Application filed October 27, 1915. Serial No. 58,232.

To all whom it may concern:

Be it known that I, HARRY W. BROADY, a citizen of the United States, and a resident of Bayside, county of Nassau, and State of New York, have invented certain new and useful Improvements in Processes and Products of Treating Wood, of which the following is a description in such full, clear, and exact terms as will enable any person skilled 10 in the art to which it pertains to make and use the same.

My invention relates to the treatment of wood by its impregnation or, more exactly, coating the interior walls of its pores or 15 inter-cellular cavities with a compound which is at once waterproof and antiseptic; and its object is to secure a mixture of waterproof and preservative materials and a mode of working with them which will 20 cause the mixture readily and completely to enter the cavities, overcome the mechanical difficulties of penetrating to the innermost recesses of the wood and form a perfect waterproof and antiseptic coat or covering 25 on the interior walls of the cells or cavities of the wood. The mixture may also, if desired, be made to seal or plug up the open or exposed outer ends of the wood cavities or pores. Such treatment not only tends to 30 prevent moisture from entering the cavities, but it coats the walls thereof so that should moisture enter it will not be absorbed by the wood fiber itself and the wood caused to take what is commonly known as a water- 35 logged condition.

The difficulty has been with the process heretofore employed that the waterproof compound fills the wood irregularly and cannot be forced into the innermost cavities 40 of the wood, particularly when the wood is treated in large pieces: it has left the outer parts of the cavities clogged with too much waterproofing and the inner parts untreated. Furthermore, it has not heretofore been 45 discovered what materials combine with the best results for these operations: various mixtures of hydrocarbons have been employed with varying, but not complete, success. This is particularly true in connection 50 with the light, spongy wood known as bal-

sade palmo, (*Ochroma lagopus*) which species of wood it is an especial object of my invention successfully to treat.

My invention seeks to solve these difficulties in the following manner: A mixture 55 of paraffin and bitumen is prepared preferably in the proportions of bitumen 25% and paraffin 75%. The bitumen is preferably asphalt. My experiments have indicated that asphalt defined as solid or semi-solid bitumen and described in the *Year Book of the American Society for Testing Materials for 1915*, published by the society is best suited to my purpose but my invention is not so 60 specifically limited. This asphalt at normal atmospheric temperatures takes a hardened 65 form, *i. e.*, a degree of hardness or firmness, not liquid or fluid but, of course, not necessarily as hard as wood, for example; and it is in this sense that the term "harden" is 70 used. The paraffin may be the ordinary paraffin of commerce. Paraffin is preferred though other materials may be employed in its place, for example, rosin. The paraffin and bitumen serve the function of a waterproof coat and both contribute water 75 resistant properties to the mixture. Further, the bitumen has an antiseptic effect on the wood which is of great value in my process. These ingredients are mixed by melting 80 them together at a temperature of approximately 130° F., at which they take liquid or viscous form and mix thoroughly. The two materials thus mixed melt at a lower temperature 85 than that of either constituent, and the resultant mixture is a stable one in which the two materials do not tend to "settle out" or separate. The materials or ingredients unite in much the same way that metals unite in alloys. The paraffin behaves somewhat 90 as a solvent of the bitumen; it has the lower melting point and appears to bring down the melting point of the bitumen.

When the hot bath is thus prepared the wood in its normal green state, or if desired 95 in cured or partly cured form is submerged in the mixture of the bitumen and paraffin and the temperature of such mixture is raised to approximately 212° to 265° F. The result is that the moisture in the wood 100

## BEST AVAILABLE COP

1,903,577

is driven off as steam and escapes in bubbles through the bath of paraffin and bitumen during and after which the mixture enters the pores and cavities of the wood. This 5 mixture of paraffin and bitumen is extremely fluid at the temperature described and readily penetrates the wood deeply, the wood appearing to have a peculiar attraction for the mixture which greatly facilitates the 10 treatment.

It is also an object of my invention to cause the mixture to spread out in a film or coat along the inner surfaces of the walls of the good cavities and not simply to plug or 15 clog up the ends or even completely to fill these cavities. These undesirable latter conditions are frequently the effect of the processes heretofore employed, *i. e.*, when the wood is treated by submersion in a hot bath 20 of ordinary waterproof compounds, part of the cell walls are coated, but in other places the mixture lies in agglomerated masses tending to fill and clog the cavities and to still other places the mixture does not reach 25 at all and the walls at these points are left untreated and hence unprotected from moisture. This is due sometimes to the size of the wood treated and the consequent remoteness of the cavities, but more generally to 30 the expansion of the gases trapped in the wood cells, which gases occupy the inner recesses and prevent the mixture from entering. I overcome this defect by treating the wood to a primary submersion which is preferably carried on until the bubbling ceases, 35 this bubbling being due to the escape of moisture (steam) and gases from the wood. The time required for the primary submersion depends upon the size and kind of wood 40 treated. It drives off part of the moisture and part of the expanded gases from the wood and effects penetration as completely as may be at that time. Then the bath is allowed to cool and harden with the wood 45 therein after which it is again heated and liquefied as before. The second heating should be continued until the wood is heated throughout; there is practically no bubbling on the second heating. By tests it has been 50 determined that this reheating required from one to six hours, according to the size and kind of wood. The mixture thereupon completes its entry into the wood and extends farther than it can be made to extend 55 by one continuous heating, no matter how long the first heating is maintained. In this way I secure one of the principal objects of my invention, *i. e.*, the thorough penetration of the wood. If desired the wood 60 may be withdrawn from the mixture after the first heating and the second heating of the wood carried out in any suitable heated chamber.

It is my opinion, based on my experiments,

that this deep penetration of the wood upon 65 heating, cooling and reheating of the mixture is due largely to the action of the gases in the pores expanding and contracting under the varying heat degrees, the gases expanding under the first heating and that 70 part which is not actually vented or driven off at the first heating contracting on the cooling so that a partial vacuum is formed in the innermost parts of the wood cavities which allows the pressure of the atmosphere 75 to force the still soft mixture farther into the wood until the mixture cools. Then on reheating the mixture enters farther into the wood and, being liquefied throughout, is allowed to flow evenly and thoroughly 80 over all of the inner surfaces of the cells, coating or lining them, *b*, without clogging or agglomerating in them. This is thought to be due to the fact that upon this reheating the gases previously entrapped will 85 again expand and force from the cells the excess of the mixture, at the same time evenly coating the cell walls.

After the wood receives this double heating in the bath described it is withdrawn 90 while the bath is yet hot, the excess of the deposited materials allowed to drain off and that remaining in the wood to cool and harden to form the permanent treatment of the wood.

Having thus described my invention, what I claim as new and desire to secure by Letters Patent of the United States is:—

1. The process of preserving wood which consists in coating or lining the walls of its 100 recesses or cavities with a fluid mixture of paraffin and bitumen and causing said mixture to harden in the wood.
2. The process of preserving wood which consists in coating or lining the walls of its 105 recesses or cavities with a fluid mixture of paraffin and asphalt and causing said mixture to harden in the wood.
3. The process of preserving wood which consists in coating or lining the walls of its 110 recesses or cavities with a fluid mixture containing bitumen and causing said mixture to harden in the wood.
4. The process of preserving wood which consists in coating or lining the walls of its 115 recesses or cavities with a fluid mixture containing asphalt and causing said mixture to harden in the wood.
5. As a new article of manufacture, wood the walls of the recesses or cavities of which 120 are coated or lined with a hardened mixture of paraffin and bitumen.
6. As a new article of manufacture, wood the walls of the recesses or cavities of which are coated or lined with a hardened mixture 125 containing bitumen.
7. As a new article of manufacture, wood the walls of the recesses or cavities of which

are coated or lined with a hardened mixture containing asphalt.

8. As a new article of manufacture, wood the walls of the recesses or cavities of which are coated or lined with a hardened mixture of asphalt and paraffin.

In testimony whereof I have hereunto

signed my name in the presence of two witnesses.

HARRY W. BROADY.

Witnesses:

ISAAC B. OWENS,  
PATRICK A. BOLGER.